

# UNITED STATES PATENT OFFICE.

JAMES O. HANDY AND ROBERT M. ISHAM, OF PITTSBURGH, PENNSYLVANIA, ASSIGNEES TO PITTSBURGH TESTING LABORATORY, OF PITTSBURGH, PENNSYLVANIA, A CORPORATION OF PENNSYLVANIA.

## METHOD OF REFINING WOOL-GREASE.

1,201,042.

Specification of Letters Patent. Patented Oct. 10, 1916.

No Drawing.

Application filed April 22, 1916. Serial No. 92,842.

To all whom it may concern:

Be it known that we, JAMES O. HANDY and ROBERT M. ISHAM, both citizens of the United States, residing at Pittsburgh, Allegheny county, Pennsylvania, have invented a new and useful Method of Refining Wool-Grease, of which the following is a full, clear, and exact description.

Our invention has relation to an improved method of refining wool grease to obtain what is known as "neutral wool grease" or "lanolin". These products are used largely in the leather industry, the lubricating oil industry, and in pharmacy.

The wool grease available for our method of treatment is of two kinds, namely: naphtha extracted grease obtained by treatment of the raw wool with naphtha, and brown wool grease, or "degras", obtained by acidification of the soapy water obtained in the usual processes of wool scouring.

The naphtha extracted grease is of a lighter color and contains less free fatty acids, while the other product contains all the fatty acids which were in the soap. Our method of refining is applicable to both these products, although we preferably use the naphtha extracted grease.

The refining problem consists in the removal of the free fatty acids, together with a small portion of the neutral grease, to produce a product which bleaches readily to a yellow color, is neutral, and which consists chiefly of the waxy portion of the original grease. This problem is a difficult one, because of the tendency of the grease when stirred with watery liquids to form a resistant emulsion therewith.

It has been usual in the prior art to first neutralize or saponify the grease by the use of an alkali (soda or potash) in an amount slightly in excess of the quantity required to combine with the free fatty acids. The next step has been the separation of the soap thus produced from the neutral wool grease which it is desired to recover. If the mixture is placed in water, or if water is added to the mixture and the mass is stirred, an emulsion will be formed even before all the soap is dissolved. The solution of the soap is also hindered by the stiff consistency of the wool grease itself.

Our invention provides a method by which the objectionable emulsification referred to

is obviated and by means of which a satisfactory product can be economically produced on a commercial scale.

In accordance with our invention the wool grease to be refined is first heated with about  $\frac{3}{2}$  per cent. of caustic soda in water solution, in a steam-jacketed kettle, or by other suitable heating means. The mixture is stirred until testing shows that there is no longer any free alkali. The mixture of soap and unsaponified wool grease thus produced is made resistant to subsequent emulsification and more easily washed free from soap by the addition at this stage of about six gallons of petrolic ether or naphtha or gasoline for each one hundred pounds of grease. Preferably the mass is allowed to cool to a temperature of approximately 100 degrees Fahrenheit before this solvent is added. The mixture is then poured upon the surface of approximately five times its volume of water, the water preferably having a temperature between 50 degrees and 60 degrees centigrade. At this stage the grease mixture should not be stirred with water, but may be moved cautiously, so as to permit the solution of a considerable quantity of the intermixed soap. After a few minutes, the water is drawn off and replaced by fresh water at about the same temperature. This procedure is repeated until the greater part of the soap is removed. A warm salt solution, preferably about a 2 per cent. solution, is then run in and is agitated with the grease, until all but a very small amount of the soap has been washed out. The removal of the soap may be hastened by using weak salt solutions instead of water previous to the running in of the final salt solution, since this further increases the resistance to emulsification. The remaining soap is then decomposed by the use of a small amount of calcium chloride solution. At this stage, the grease has absorbed a considerable amount of water, although it has not formed an emulsion. It also contains a small amount of lime soap. The grease must therefore be dried before bleaching.

The water is preferably eliminated by adding petrolic ether, and distilling up to a temperature where the water passes over with the solvent. The grease is then cooled and is ready for bleaching. This bleaching

may be carried out by any known method. We prefer, however, to employ the method which is described and claimed in the co-pending application of James O. Handy, one of the applicants herein, Serial No. 92,845, filed April 22, 1916. In accordance with that method the grease is dissolved in petrolic ether and is agitated with fullers' earth. By this method we secure a bleaching effect which it is impossible to obtain by treatment of the grease alone with fullers' earth. Instead of disposing of the water by distillation of the wet grease before bleaching, the grease may be dried by adding sufficient fullers' earth to absorb the water, and then heating in pans in a drying oven at a temperature of from 100 degrees to 110 degrees centigrade. The dry material is then agitated with petrolic ether and filtered. In either case the grease may be recovered from the petrolic ether solution by distilling off the solvent in a suitable form of still—preferably a still having a closed steam coil and a condensing attachment. The petrolic ether is then ready for further use.

The recovered grease may be freed from petroleum odors by blowing it with air or other suitable gas at a temperature of from 90 degrees to 100 degrees C.

The product produced is a highly satisfactory one, being perfectly neutral, is of the desired yellow color when bleached, and consists mainly of the waxy portion of the original grease. The treatment with petrolic ether for the purpose of making the mixture of soap and unsaponified wool grease more resistant to emulsification greatly simplifies the subsequent separation of the neutral wool grease from the soap.

We do not desire to limit ourselves to the precise method which we have herein shown and described, since changes may be made in the different steps thereof and in the different temperatures named, without departing from the spirit and scope of our invention as defined in the appended claims.

By the term "petrolic ether" as used herein and in the appended claims, we intend to include naphtha, gasoline, and all similar petroleum products having a sufficiently low boiling point. The boiling point should not be sufficiently low to cause losses, and, on the other hand, it should not be sufficiently high to give undesirable residual products under the conditions of evaporation employed. In practice we have found a boiling point of from 70 degrees to 100 degrees C., and preferably between 80 degrees and 100 degrees C., to give good results.

We claim:

1. In the art of refining wool grease, the improvement which consists in saponifying the free fatty acids in the grease, then preventing emulsification by adding petrolic ether to the mixture of soap and unsaponi-

fied wool grease before attempting to separate from each other the soap and the unsaponified wool grease, and then separating the soap from the unsaponified wool grease, substantially as described.

2. In the art of refining wool grease, the method which consists in saponifying the free fatty acids in the grease, permitting the mixture of soap and unsaponified wool grease to partially cool, then before attempting to separate from each other the soap and unsaponified wool grease adding thereto a solvent which renders the mixture more resistant to subsequent emulsification and more easily freed from its soap, and then separating the soap from the unsaponified wool grease by means of an aqueous liquid, substantially as described.

3. In the art of refining wool grease, the method which consists in saponifying the free fatty acids in the grease, permitting the mixture of soap and unsaponified wool grease to partially cool, then before attempting to separate from each other the soap and the unsaponified wool grease adding thereto a solvent which renders the mixture more resistant to subsequent emulsification and more easily freed from its soap, and then separating the soap from the unsaponified wool grease by means of an aqueous liquid, substantially as described.

4. In the art of refining wool grease, the method which consists in saponifying the free fatty acids in the grease, then preventing emulsification by adding petrolic ether to the mixture of soap and unsaponified grease before attempting to separate from each other the soap and the unsaponified wool grease, and then washing the mixture free from soap, substantially as described.

5. In the art of refining wool grease, the method which consists in saponifying the free fatty acids in the grease, then preventing emulsification by adding petrolic ether to the mixture of soap and unsaponified grease before attempting to separate from each other the soap and the unsaponified wool grease, and then washing the mixture free from soap by the use of a weak salt solution, substantially as described.

6. In the art of refining wool grease, the method which consists in saponifying the free fatty acids in the grease, then preventing emulsification by adding petrolic ether to the mixture of soap and unsaponified grease, before attempting to separate from each other the soap and the unsaponified wool grease, and then washing the mixture free from soap by the use of a weak salt solution and a calcium chlorid solution, substantially as described.

7. In the art of refining wool grease, the method which consists in treating the grease to produce a mixture of soap and unsaponified wool grease, then rendering this mix-

ture resistant to subsequent emulsification before attempting to separate from each other the soap and the unsaponified wool grease, and then washing the soap from the 5 mixture by means of an aqueous liquid, substantially as described.

8. In the art of refining wool grease, the method which consists in treating the grease to produce a mixture of soap and unsaponified grease, then, before attempting to separate from each other the soap and the unsaponified wool grease, rendering such mixture resistant to subsequent emulsification by the addition of a solvent, then washing the soap from the mixture, and then drying and bleaching, substantially as described.

9. In the art of refining wool grease, the method which consists in treating the grease 20 to produce a mixture of soap and unsaponified grease, then adding petrolic ether to this mixture, then pouring the mixture upon the surface of a volume of water to permit the solution of a part of the intermixed 25 soap, and then removing the water and agitating the mixture with a weak salt solution, substantially as described.

10. In the art of refining wool grease, the method which consists in treating the grease 30 to produce a mixture of soap and unsaponified grease, then adding petrolic ether to this mixture, then pouring the mixture upon the surface of a volume of water to permit the solution of a part of the intermixed 35 soap, and then removing the water and agitating the mixture with a weak salt solution and decomposing the remainder of the soap by a calcium chlorid solution, substantially as described.

40 11. In the art of refining wool grease, the method which consists in treating the grease to produce a mixture of soap and unsaponified grease, then adding thereto petrolic ether before attempting to separate from each other the soap and the unsaponified 45 wool grease, then removing the soap from the mixture, and then eliminating the water absorbed by the grease during the removal of the soap by adding a solvent and distilling at a temperature at which the water 50 will pass over with the solvent, substantially as described.

12. In the art of refining wool grease, the

method which consists in treating the grease to produce a mixture of soap and unsaponified 55 grease, then adding thereto petrolic ether before attempting to separate from each other the soap and the unsaponified wool grease, then removing the soap from the mixture, and then eliminating the water absorbed by the grease during the removal of the soap by adding petrolic ether and distilling at a temperature at which the water 60 will pass over with the petrolic ether, substantially as described.

65 13. In the art of refining wool grease, the method which consists in saponifying the free fatty acids in the grease, then adding petrolic ether to the mixture of soap and unsaponified grease, and floating the mixture 70 on water, without agitation, to remove the soap therefrom, substantially as described.

14. In the art of refining wool grease, the method which consists in saponifying the 75 free fatty acids in the grease, then adding petrolic ether to the mixture of soap and unsaponified grease, and floating the mixture 80 on a weak salt solution, substantially as described.

85 15. In the art of refining wool grease, the method which consists in saponifying the free fatty acids in the grease, then adding to the mixture of soap and unsaponified grease a solvent which will render the mixture more resistant to subsequent emulsification, then floating the mixture on water to remove the soap therefrom, substantially as described.

90 16. In the art of refining wool grease, the method which consists in saponifying the free fatty acids in the grease, then adding to the mixture of soap and unsaponified grease a solvent which will render the mixture more resistant to subsequent emulsification, and then floating the mixture on a 95 weak salt solution, substantially as described.

In testimony whereof, we have hereunto set our hands.

JAMES O. HANDY.  
ROBERT M. ISHAM.

Witnesses:

W. C. LYON,  
H. M. CORWIN.